

## UNITED STATES PATENT OFFICE

2,380,878

AGENTS FOR LUBRICATING OILS AND  
METHODS OF MAKING THE SAME

Herschel G. Smith, Wallingford, and Troy L. Cantrell, Lansdowne, Pa., assignors to Gulf Oil Corporation, Pittsburgh, Pa., a corporation of Pennsylvania

No Drawing. Application July 3, 1943,  
Serial No. 493,898

10 Claims. (Cl. 252—32.7)

This invention relates to improvement agents for lubricating oils and methods of making the same.

In the lubrication of internal combustion engines of all types, particularly when severe operating conditions are encountered, plain mineral oils often prove unsatisfactory, due to the attendant deposition on the engine surfaces, such as cylinder walls, pistons and rings, of "varnish," gum or "sludge." This effect is particularly serious in modern engines operating under severe conditions, such as Diesel engines, aviation, truck and tank engines. The problem has become increasingly serious, due to the trend toward higher efficiency, higher power out-put per unit weight per engine, reduction in the amount of oil employed in the lubrication system of the engine, and other conditions which tend to accelerate the deteriorating influences on mineral lubricating oil.

Formation of so-called varnishes and sludges on engine surfaces is due to oxidation or polymerization effects (or both) of the lubricating oils, as well as to like effects of or from products of combustion of the fuels, which find their way by leakage into the engine crankcase or other parts of the engine.

The presence of these substances is disadvantageous for many reasons. In particular, the oil and fuel oxidation products tend to increase ring sticking and production of deposits on piston surfaces and in fixed parts of the combustion chamber. Sludges are formed in the crankcase of the engine, and the rate of corrosion of bearing surfaces is increased, especially with bearing alloys of the types now in use.

Petroleum oils intended for use under the severe conditions described are compounded (almost always) with a mixture of substances each intended to counteract one or more of the undesirable effects noted. These substances, which fall into a wide variety of chemical classifications, are known by the general term "improvement agents" or addition agents. Preparation of satisfactory compounded lubricants is a matter of considerable difficulty. Some of the agents are of low potency in that a rather large amount has to be added to achieve the desired result. Often two or more agents are more or less incompatible with each other; and their rather low solubility, in general, further adds to the difficulties in preparing a useful lubricant.

One object of the present invention is the provision of an improvement agent for engine oils which can be incorporated in petroleum oils in

effective proportions and which imparts to the oil a plurality of functions.

Another object is the provision of such an agent in the form of a solution in petroleum lubricating oils which serves the functions of (1) acting as a negative catalyst to suppress the formation of deterioration or oxidation products, such as varnish, sludge and gum, (2) acting as loosening or suspending agent (detergent) to prevent ring sticking, "varnishing," or coating of metallic surfaces by such reduced amounts of deterioration products as may be formed and (3) acting as a suspending or dispersing agent for retaining very small particles of solid deterioration or contaminating materials in the oil; for example, particles of carbonaceous matter that find their way into the crankcase oil by passing the piston rings which cannot possibly be made absolutely tight.

20 Another object is the provision of a new improvement agent capable of increasing the solubility or dispersibility of other agents, such as straight soaps or the like, when it is desirable also to add such compounds to an oil in which said soaps and like agents are difficultly soluble.

According to this invention, new improvement agents for lubricating oils capable of achieving these and other objects are prepared from certain alkylated phenols (olefin-phenol reaction products) by simultaneously reacting phosphorus trichloride (PCl<sub>3</sub>) and phosphorus sesquisulfide (P<sub>2</sub>S<sub>3</sub>) with the alkylated phenols to form complex acid reaction products which, in turn, are treated with lime (or other metal oxide or hydroxide) producing stable metallo-compounds of alkylated phenol esters of phosphorus acids of the character described in more detail below. That is, as shown post, the new agents are prepared from alkylated phenols containing at least one branched-chain alkyl group. Likewise, as there shown, in preparing our new agents, such alkylated phenols are simultaneously reacted with phosphorus trichloride and phosphorus sesquisulfide under controlled conditions to produce acid reaction products thereof, and the acid reaction products so obtained are heated with polyvalent metal oxides or hydroxides until stable, substantially neutral metallo-derivatives thereof are obtained, the stable oil-soluble improvement agents so obtained being separated from the unreacted metal oxides and hydroxides and other insoluble compounds. The polyvalent metal compounds so obtained, particularly the di- and tri-valent compounds and mixtures thereof, are useful and advantageous for the present purposes.

The so-prepared agents or metallo compounds, in solution in lubricating oils, provide four functions which are useful and advantageous in lubricants: (1) by virtue of its combined metal (e. g. calcium, etc.) suspending or detergent properties are imparted, as well as resistance to ring sticking; (2) the combined phosphorus imparts anti-bearing-corrosion and anti-ring sticking properties, as well as pressure carrying properties; (3) the combined sulfur serves to give pressure carrying properties to the oil and to retard corrosion of alloy bearings and (4) by virtue of the organic nucleus, the alkylated phenyl groups carrying at least one branched chain alkyl group, the improved oil has good antioxidant and oiliness properties and suspending and solubilizing characteristics.

Thus, according to the invention, there is provided a compound which, dissolved in the oil, imparts thereto all the many desirable features which we wish to obtain, including the several advantages, virtues and properties described ante. Further, our new improvement agents are so soluble in motor oils of all types and degrees of refinement that we can incorporate them in any desired proportions to form a clear solution in lubricating oils, even in the most highly refined and most paraffinic of the heavy aviation oils, such as are specified in the most severe and exacting aviation services.

It is known that highly paraffinic oils, refined to the high degree desired to secure such desired properties as low carbon-forming effects and high viscosity indices (improved viscosity temperature relationships) are relatively poor solvents for decomposition products formed in use. Also there is increased tendency to induce bearing corrosion. In this invention these undesirable properties of such oil are done away with by the use of moderate amounts of our new compounding agent having cumulatively all the desired properties in the way of ready solubility in the oils and the other advantageous effects mentioned above. We can employ very highly refined paraffinic-type aviation oils that have the desired superior physical characteristics as regards these particular properties, and, at the same time, avoid any undesirable effects whatever from the use of such oils. In other words, the addition of our compound, which is soluble in the heavy highly refined paraffinic oils, enables us to secure all the properties desirable in the way of the oils of superior performance characteristics, as well as the effects of detergency, avoidance of ring sticking, varnish formation, sludge formation and corrosion of alloy bearings that might otherwise be encountered, as well as secure the desired effect of retarding oxidation due to the use of more highly refined oils of less tendency to oxidize combined with the use of a compound which actually retards oxidation.

Another important field of utility for the invention is in Diesel lubricating oils. Heretofore, it has been considered best to use naphthene-type oils dosed with certain compounding agents which are of undesirably low efficiency and which, moreover, are not readily soluble even in the most naphthenic type of Coastal oils. Thus it has often been necessary to make a compromise even for the Coastal oils of greater solubility effect for compound agents between the degree of refining and the solubility effect for the addition agents. It is quite unsatisfactory for most of these agents to use even a moderately refined paraffin-type oil, as all or part of the addition agents heretofore

used will often separate from the oil upon standing. For these reasons Diesel lubricating oils hitherto prepared have been rather unsatisfactory, in that they employ low grade oils of less degree of resistance to oxidation than would otherwise be desirable. With the present invention, we prepare an improved oil which performs satisfactorily in Diesel engines, employing a highly refined paraffin-type of oil with control of ring sticking effects and sludge formation and detergency effects by the incorporation of the present compound in any desired proportion.

The new improvement agent has another important advantage in that, in addition to being very oil-soluble itself, it acts to disperse in mineral oils other improvement agents which are of themselves relatively insoluble. For example, in accordance with the present invention, one percent or more of calcium oleate or aluminum stearate can be dispersed in mineral oil to form a stable and permanent dispersion with the aid of an equal quantity of the new agent. Thus, the new agent is sometimes useful when and where its own antioxidant and dispersing properties are not required for its value in dissolving other agents.

The new agent is conveniently prepared in the form of a concentrated oil solution which can readily be stirred into an oil to prepare a compound lubricant. In preparing the new agent, the base material is advantageously alkylated phenols which themselves have good antioxidant properties. A convenient source for this base material or principal reactant is the phenol-olefin reaction products prepared as described in U. S. Patent 2,149,759, issued March 7, 1939, to Troy Lee Cantrell. For instance, an advantageous material is a "heart-cut" of such phenol-olefin reaction products, prepared from the 20-80 per cent cut separated by steam or vacuum distillation; vacuum distillation being preferred. This heart-cut is a mixture of liquid, semi-liquid and crystalline alkylated phenols. It is soluble in all proportions in lubricating oils and gasoline, and soluble in most organic solvents and insoluble in water and NaOH solutions. It has the following properties:

|                              |               |
|------------------------------|---------------|
| Gravity: ° A. P. I.          | 18.0-24.0     |
| Sp. Gr., 60°/60° F.          | 0.9465-0.9100 |
| Viscosity, S. U. V.: 100° F. | 61-100        |
| Pour: ° F.                   | -30 to +15    |
| Color, N. P. A.              | 1.0-1.5       |
| Free phenol: per cent        | Nil           |
| Mineral acidity: per cent:   |               |
| SO <sub>3</sub> equivalent   | Nil           |
| Distillation, ASTM D 86-40:  |               |
| Over point: ° F.             | 375-380       |
| End point: ° F.              | 525-540       |
| 10 per cent at: ° F.         | 415-450       |
| 50                           | 470-495       |
| 90                           | 495-525       |

This phenol-olefin reaction product contains varying amounts of 4-tertiary-butyl-phenol, 2-tertiary-butyl-4-secondary-butyl phenol, 2,4-di-tertiary-butyl phenol, 2,6-di-tertiary-butyl-4-secondary-butyl phenol, 2,4,6-tri-tertiary-butyl phenol, 2,6-di-tertiary-butyl-4-methyl phenol, 4,6-di-tertiary-butyl-2-methyl phenol, 4,6-di-tertiary-butyl-2-methyl phenol, and other alkylated phenols containing a branched chain alkyl group attached to the phenyl nucleus thereof. All these alkylated phenols have good antioxidant properties and are useful in making our

new improvement agents. As a class they may be represented by the following generic formula



wherein R, R' and R'' represent hydrogen or an alkyl group, at least one branched chain alkyl group being present. Those containing secondary or tertiary alkyl groups are particularly advantageous for the present purposes.

In proceeding in accordance with the first stage of the present invention, such alkylated phenols are brought into reaction with phosphorus trichloride and phosphorus sesquisulfide in the desired proportions, the mixture of reactants being heated to facilitate reaction. Upon heating the mixture, the three reactants vigorously interact, forming complex alkylated phenyl esters of phosphorus acids, wherein the alkylated phenyl groups thereof contain at least one branched chain alkyl substituent. Advantageously, the reaction may be effected at temperatures between 300° and 540° F. and is usually carried out at about 420° F. Likewise, the proportions of the reactants, namely the alkylated phenols, phosphorus trichloride (PCl<sub>3</sub>) and phosphorus sesquisulfide (P<sub>4</sub>S<sub>3</sub>), may be varied and controlled to produce reaction products advantageous for the present purposes. Usually we employ 10 to 40 parts of phosphorus trichloride and 0.1 to 10.0 parts of phosphorus sesquisulfide per 100 parts of the alkylated phenol. The acid reaction products so obtained readily react with metal oxides and hydroxides, forming metal salts of these alkylated phenol esters.

In forming such metal salts, the acid reaction products or esters described ante may be heated with various polyvalent metal oxides and hydroxides, the reaction mixture being heated to temperatures between 300° and 450° F. until stable, substantially neutral, oil-soluble metallo derivatives of said acid reaction products are obtained. During this heating complex reactions occur and the acid reaction products or esters are converted into stable, neutral, oil-soluble metallo compounds which are useful as improvement agents in mineral oils and oil composition and are stable under the service conditions usually encountered by commercial lubricants. That is, this heating in the presence of metal oxide or hydroxide stabilizes the improvement agent at the time it is formed.

After the reaction is complete, any excess metal oxide or hydroxide and insoluble by-products are separated from the improvement agent by settling, filtration or other suitable method. Usually these oil-soluble metallo compounds or improvement agents, with or without dilution with mineral oils, are filtered to remove insoluble materials. The filtrates are then ready for use in accordance with this invention.

For instance, valuable improvement agents are readily obtained by heating such acid reaction products or esters with lime. In doing so, lime (quick or hydrated) is added in the proportions of about 10 to 30 parts (figured on CaO) per 100 parts of reaction products and the mixture heated at a temperature of 325° to 400° F. for about 5 hours. The reaction mixture is filtered and is ready for use. By adding mineral oil to

the above reaction mixture prior to the heating, concentrated solutions of the improvement agent in oil can be directly obtained upon filtering out the insoluble material.

5 In lieu of ordinary lime, dolomitic limes, magnesia or magnesium hydroxide can be employed. Likewise, other polyvalent metallic oxides or hydroxides, such as alumina or zinc oxide may be employed in preparing our metallo-derivatives or metal salts of these alkylated phenyl esters of phosphorus acids. That is, various metal compounds may be employed in the practice of this invention.

The improvement agents so obtained are of complex constitution, even when a single alkylated phenol, such as 2,6-di-tertiary-butyl-4-methyl phenol, etc., is employed. Further, using mixtures of alkylated phenols, such as the "heart-out" of the olefin-phenol reaction products described ante, mixtures of metallo-derivatives of alkylated phenyl esters are obtained. As stated, these are advantageous in the practice of this invention.

That is, our improvement agent is probably a mixture of similar or analogous compounds and may contain varying proportions of the several constituents, namely combined phosphorus, sulfur, metal, etc., combined in a complex metallo compound. As a matter of fact, we vary the relative proportions of the reactants, depending upon the particular properties desired. There is considerable flexibility in the proportion of calcium or other metal added and combined for securing a range of detergency, anti-ring sticking, and 25 solid suspension effects; or in the amount of combined phosphorus as required to obtain the desired anti-ring sticking and anti-corrosion effects. That is, these constituents of our improvement agents can be varied at will. For instance, the metal content can be made to vary over relatively wide limits.

30 That is, in practice we vary the proportions of the several reactants in accordance with the particular properties desired. After the desired 35 combinations have been effected, the reaction product is filtered to remove insoluble compounds and is then ready for use. The filtered materials are readily soluble in lubricating oil.

In preparing improved lubricants, the optimum 40 proportion of the agent to be introduced into lubricating oils depends on the severity of the service conditions and the degree to which the oil itself tends to form gum or varnish. Ordinarily, from 0.1 to 5.0 per cent by weight of the improvement agent on the oil is suitable. The improved lubricants so obtained have the advantageous properties described ante and are superior lubricants.

45 The preparation and use of our improvement agents is further illustrated in the following illustrative examples which are typical but not limitative of this invention.

Example 1.—In this specific example illustrative of one advantageous way of preparing an agent within the purview of this invention, 1238 pounds of the above described phenol-olefine reaction product were heated to 100-120° F. in a stirring still and 412 pounds of phosphorus trichloride and 4.5 pounds of phosphorus sesquisulfide were gradually added with stirring. After 5 hours at this temperature, the temperature was gradually raised and held to 410-420° F. for a period of 24 hours.

50 The reaction product so obtained was a mixture

of alkylated phenyl esters of phosphorus acids and had the following properties:

|                              |      |
|------------------------------|------|
| Gravity                      | 9.0  |
| Viscosity, S. U. V.: 100° F. | 560  |
| Color, N. P. A.              | 1.75 |
| Phosphorus: per cent         | 5.92 |
| Chlorine: per cent           | 7.60 |

It readily reacts with metal oxides and hydroxides forming metal derivatives.

In forming stable substantially neutral calcium derivatives thereof, 1200 pounds of the above reaction product were heated with 222 pounds of lime in water at 170° F. The mixture was then gradually heated to 325° F. and maintained at this temperature for five hours. The resulting product was cooled to 250° F. and filtered to remove excess lime and other insolubles.

The calcium treated product so obtained had the following properties:

|                              |      |
|------------------------------|------|
| Gravity: ° A. P. I.          | 11.2 |
| Viscosity, S. U. V.: 210° F. | 150  |
| Ash as sulfate: per cent     | 8.3  |

The above product was readily soluble in mineral lubricating oils. It is an excellent improvement agent for such oils and imparts to them the several advantageous improvements described ante.

By adding varying proportions of this improvement agent to commercial lubricating oils, a wide range of improved lubricants is readily obtained.

Further, the improvement agent prepared in Example 1 ante, is so soluble in mineral oils that concentrated solutions thereof can be readily prepared. These concentrates are also useful improvement agents in making commercial lubricants and can be readily incorporated and blended with various lubricating oils and bases to produce commercial lubricants.

These concentrates can also be prepared with advantage by incorporating mineral oil with the acid reaction product prior to reacting the same with the metal oxide or hydroxide. One such advantageous embodiment of this invention is illustrated in the following example:

*Example 2.*—In this specific example illustrative of another advantageous way of preparing our improvement agents, 880 pounds of the above described phenol-olefin reaction product were heated to 100-120° F. and 10 pounds of P<sub>4</sub>S<sub>3</sub> and 274 pounds of PCl<sub>3</sub> were gradually added. After five hours at this temperature, the temperature was gradually raised and held at 450° F. for a period of 18 hours.

The reaction product so obtained was a mixture of alkylated phenyl esters of phosphorus acids and had the following properties:

|                              |        |
|------------------------------|--------|
| Gravity: ° A. P. I.          | 11.0   |
| Specific gravity, 60°/60° F. | 0.9930 |
| Viscosity, S. U. V.: 100° F. | 530    |
| Color, N. P. A.              | 1.75   |
| Sulfur, Carius: per cent     | 1.25   |
| Chlorine, Carius: per cent   | 8.60   |
| Phosphorus: per cent         | 5.91   |

This reaction product was diluted with approximately an equal weight of mineral lubricating oil, namely, a Texas oil having a Saybolt viscosity of 104 at 100° F. The mixture containing 500 pounds of the reaction product and 500 pounds of mineral oil was stirred in an open iron vessel and 74 pounds of hydrated lime added.

This mixture was agitated and heated to 350° F. for 5 hours. The solution of improved agent in oil so obtained was then admixed with a filter aid and filtered.

The filtrate had the following identified properties:

|                              |        |
|------------------------------|--------|
| Gravity: ° A. P. I.          | 17.5   |
| Specific gravity, 60°/60° F. | 0.9497 |
| Viscosity, S. U. V.:         |        |
| 100° F.                      | 235    |
| 210° F.                      | 44.2   |
| Pour: ° F.                   | —20    |
| Color, N. P. A.              | 2.5    |
| Sulfur, B: per cent          | 0.56   |
| Chlorine, Carius: per cent   | 0.15   |
| Phosphorus, Carius: per cent | 2.85   |
| Carbon residue: per cent     | 2.4    |
| Ash as sulfate: per cent     | 4.0    |

It is an excellent improvement agent for lubricating oils; it being a concentrated solution of the effective agent in oil.

By adding varying proportions of this concentrate to commercial lubricating oils, a wide range of improved lubricants is readily obtained.

In the foregoing examples, other polyvalent metal oxides or hydroxides may be employed in lieu of lime and other polyvalent metal salts obtained which are likewise excellent improvement agents for mineral lubricating oils. They too are readily soluble in both paraffinic and naphthenic oils and can be readily incorporated and blended with all types of commercial lubricating oils to obtain improved lubricants. The preparation of such improved lubricants is further illustrated in the following examples:

*Example 3.*—An improved lubricating oil was prepared by dissolving 1 per cent of the preparation of Example 1 in a high grade lubricating oil for use in Diesel engines.

*Example 4.*—An improved lubricating oil was prepared by dissolving 2 per cent of the preparation of Example 2 in a high grade lubricating oil for use in Diesel engines.

The viscosities and conventional identifying characteristics of these improved lubricating compositions, together with those of the base oil, were as follows:

| Properties                 | Base oil | Improved lubricant |           |
|----------------------------|----------|--------------------|-----------|
|                            |          | Example 3          | Example 4 |
| Gravity: ° API             | 22.2     | 21.9               | 28.2      |
| Viscosity, S.U.V.: 100° F. | 510      | 497                | 564       |
| Flash, OC: ° F.            | 385      | 380                | 460       |
| Fire, OC: ° F.             | 440      | 425                | 530       |
| Pour: ° F.                 | —10      | —5                 | 0         |
| Color, N.P.A.              | 3.0      | 3.25               | 4.0       |
| Carbon residue: Percent    | 0.09     | 0.07               | 0.11      |

In order to evaluate their tendency to prevent ring sticking in engines, these compositions were subjected to a motor test in the laboratory, using a standard Waukesha-CFR crankcase with special L head type cylinder block, coupled to a cradle-type electric dynamometer. This engine has a bore of 3 1/4 inches, a stroke of 4 1/2 inches, and a compression ratio of 4.7:1. The piston is of cast iron with four compression rings and one oil-control ring, all located above the wrist pin. Three liters of the oil to be tested are placed in the crankcase. The engine is then run at 900 R. P. M. with the spark and the air-fuel ratio adjusted to give maximum power, and the coolant temperature is maintained at 350° F. At the end of 25 hours' running, the engine is stopped and

dismantled and the piston is examined. The performance of the oil is then rated according to the condition of the piston, in keeping with the following scale, in which the rating number increases as the piston condition becomes worse:

*Ratings:*

- No. 1—No rings stuck, and no heavy hard deposits.
- No. 2—Top or oil ring (or both) stuck on a small part of circumference.
- No. 3—Top or oil ring (or both) completely stuck,
- No. 4—Top or oil ring (or both) completely stuck and ring partly stuck,
- No. 5—Top, 2nd, and oil rings completely stuck,
- No. 6—Condition No. 5 with 3rd, and 4th rings partly stuck.

In the above test the rating of the several compositions were as follows:

| Composition     | Base oil | Improved oil |           |
|-----------------|----------|--------------|-----------|
|                 |          | Example 3    | Example 4 |
| Rating No. .... | 4        | 2            | 1         |

These compositions were also subjected to the well known Almen and Timken lubricating test with the following results:

| Composition              | Base oil | Improved oil |           |
|--------------------------|----------|--------------|-----------|
|                          |          | Example 3    | Example 4 |
| Almen test, ..... pounds | 6        | 18           | 24        |
| Timken test, ..... do    | 14       | 20           | 30        |

Similar improved results are obtained with lubricating oils containing small amounts of other polyvalent metal salts of these esters of alkylated phenols.

While the improvement agent of the present invention has been described in reference to compounding engine lubricating oils for the primary purpose of preventing ring sticking, its field of usefulness is not confined to that application. It can be used in oils wherever its properties may be desired. Sometimes it is used for its dispersive powers on other agents, when its own antioxidant and detergent properties are not needed.

That is, another important advantage of the agents of the present invention is that in addition to being highly soluble in oils themselves, they are effective to disperse in mineral oils certain soaps which are of themselves difficultly soluble, for example, calcium oleate or aluminum stearate. Again, sulfurized sperm oil soap is a desirable addition agent to oils, but its low solubility prevents incorporation of more than a rather small quantity in paraffin base oils. By the present invention 1 per cent or more of such soap can be dispersed in oil, to form a stable dispersion by including an equal amount of the new improvement agents of this invention. Thus in the practice of the present invention, our new agents may be used in conjunction with other previously known addition agents, in compounding lubricating oils to improve their properties. Thus in the practice of the present invention, various embodiments thereof may be employed in addition to the illustrative embodiments shown ante.

What is claimed is:

1. A process of preparing an improvement agent for lubricating oils, from alkylated phenols containing at least one branched chain alkyl group, which comprises heating 100 parts of said alkylated phenols with 10 to 40 parts of phosphorus trichloride and 0.1 to 10 parts of phosphorus sesquisulfide, by weight, at temperatures between 300° and 540° F. until substantially all of the phosphorus trichloride and phosphorus sesquisulfide have reacted and acid reaction products thereof are obtained, and converting the acid reaction products so obtained into stable, substantially neutral metal derivatives thereof by further heating said acid reaction products with a reactive metal compound of a class consisting of the oxides and hydroxides of a polyvalent metal, the amount of said reactive polyvalent metal compound being sufficient to neutralize the acidity of said reaction products, and the mixture being heated to temperatures between 300° and 450° F. until stable, substantially neutral metal derivatives thereof are obtained, and separating the unreacted metal oxides and hydroxides and other insoluble compounds from the oil-soluble improvement agent so obtained.
2. The method of claim 1 wherein said reactive metal compound is lime.
3. The method of claim 1 wherein said reactive metal compound is a divalent metal compound.
4. The method of claim 1 wherein the alkylated phenols employed as the starting material are phenol-olefin reaction products comprising a mixture of alkylated phenols containing secondary and tertiary alkyl groups.
5. The method of claim 1 wherein the said acid reaction products of the alkylated phenols are heated with the said polyvalent metal compounds in proportions of 10 to 30 parts of the reactive metal compound per 100 parts of said acid reaction products.
6. The method of claim 1 wherein said acid reaction products are diluted with mineral oil prior to the treatment with the said polyvalent metal compounds, and wherein the oil solution of stable, substantially neutral oil-soluble metallo compounds so obtained are filtered to remove unreacted metal oxides and hydroxides and other insoluble compounds.
7. A process of preparing an improvement agent for lubricating oils, from alkylated phenols containing at least one branched chain alkyl group which comprises heating 100 parts of said alkylated phenols with 10 to 40 parts of phosphorus trichloride and 0.1 to 10 parts of phosphorus sesquisulfide, by weight, at temperatures between 300° and 540° F. until substantially all of the phosphorus trichloride and phosphorus sesquisulfide have reacted and acid reaction products thereof are obtained, diluting the acid reaction product so obtained with mineral oil, adding to the so fluxed acid reaction products a reactive metal compound of the class consisting of the oxides and hydroxides of a polyvalent metal in proportions of 10 to 30 parts of said reactive metal compound per 100 parts of said acid reaction products, further heating the mixture to temperatures between 300° and 450° F. until stable, substantially neutral, oil-soluble metallo derivatives thereof are formed in situ in the mineral oil, and filtering the oil concentrate of the improvement agent so obtained to remove unreacted metal oxides and hydroxides and other compounds insoluble in the oil.

8. An improvement agent soluble in petroleum oil and capable of inhibiting formation of gum, varnish, and sludge in engines, comprising the stable, oil-soluble, substantially neutral metallo compounds obtained by the process of claim 1.
9. An improved lubricating composition comprising a major amount of a mineral lubricating oil and a small proportion of the stable, oil-soluble, substantially neutral metallo compounds obtained by the process of claim 1, the amount 10 of said oil-soluble improvement agent being suffi-

cient to inhibit the formation and deposition of gum, varnish and sludge in engines and to disperse such deposits when present.

10. An improvement agent, for lubricating oils, comprising the stable, substantially neutral product of the process of claim 7, said product being readily soluble in petroleum oils and capable of inhibiting formation of gum, varnish and sludge in engines.

HERSCHEL G. SMITH.  
TROY L. CANTRELL.